

# UNITED STATES PATENT OFFICE.

JOHN B. DEEDS, OF TERRE HAUTE, INDIANA, ASSIGNOR TO ROBERT H. CATLIN, OF SAME PLACE.

## ANTI-FRICTION COMPOUND.

SPECIFICATION forming part of Letters Patent No. 395,216, dated December 25, 1888.

Application filed February 11, 1888. Serial No. 263,674. (Specimens.)

*To all whom it may concern:*

Be it known that I, JOHN B. DEEDS, a citizen of the United States, residing at Terre Haute, in the county of Vigo and State of Indiana, 5 have invented certain new and useful Improvements in Packing Compounds; and I do hereby declare the following to be a full, clear, and exact description of the invention, such as will enable others skilled in the art to 10 which it appertains to make and use the same.

This invention relates to certain new and useful improvements in materials or compounds designed as a lining or packing for stuffing-boxes, journal - bearings, machine-joints, and similar uses.

The object of the invention is to supply a compound which shall possess the characteristics of durability and compactness by which to render the same of considerable value for 20 the purposes intended.

In carrying my invention into effect I take about one pound of tallow or similar fatty matter, and to this I add about two ounces of beeswax or paraffine, and these are placed in 25 any suitable vessel and heated very hot, so as to become melted and intimately mixed. A constant stirring of the mixture should be kept up, and when sufficiently mixed I add about three ounces of plumbago or black lead 30 combined with an equal amount of brimstone, and also stir this up thoroughly. All should be kept heated for at least one hour, after which I add to the heated mixture about one-half pound of asbestos yarn or wicking combined 35 with as much strong hemp as will absorb the heated mixture, which, when saturated and

permitted to cool, will act to hold the mass together strongly when subjected to a high pressure or great friction. No further mode of compounding is necessary.

I have used a compound thus prepared, and have found it to possess all the requirements of a packing for stuffing-boxes, joints, and the like, and I have also found that when the fibers of asbestos and hemp have become thus 45 treated the resultant compound or material may be readily twisted or plaited into a rope of any desired size or length. When used as a packing for stuffing-boxes, I have found it very valuable for filling the space within the 50 stuffing-box surrounding the metallic ring described and claimed in my application of even date herewith, Serial No. 263,725; but it is evident that I am not limited to such use.

Having thus described my invention, what I 55 claim as new, and desire to secure by Letters Patent, is—

A lining or packing consisting of the following ingredients in about the proportions named: one pound of tallow or similar fatty 60 matter, two ounces of beeswax or paraffine, three ounces of plumbago combined with about an equal quantity of brimstone, one-half pound of asbestos yarn or wicking, and strong hemp, substantially as described.

In testimony whereof I affix my signature in presence of two witnesses.

JOHN B. DEEDS.

Witnesses:

WILLIAM DIDRISH,  
JOHN R. TAYLOR.